

May 26, 1942.

W. G. WEHR

2,284,240

RAIL FOR OVERHEAD MONORAIL CARRIER SYSTEMS

Filed April 26, 1940



FIG. 1



FIG. 2

INVENTOR.

BY WILLIAM G. WEHR

Kris Hudson & Kent  
ATTORNEYS

## UNITED STATES PATENT OFFICE

2,284,240

## RAIL FOR OVERHEAD MONORAIL CARRIER SYSTEMS

William G. Wehr, East Cleveland, Ohio, assignor to The Cleveland Crane & Engineering Company, Wickliffe, Ohio, a corporation of Ohio

Application April 26, 1940, Serial No. 331,766

5 Claims. (Cl. 104—109)

This invention relates to a track rail for overhead monorail underslung carrier systems and has for its chief object to provide increased safety by reducing the likelihood of breakage of the rail and person or persons thereunder being injured by a falling load or carrier, and at the same time to provide increased life by improved wearing qualities of the tread surfaces which are engaged by the wheels of the carriers. In brief, the invention aims to successfully solve the users' requirements for constantly increasing tonnage and speed conditions of overhead monorail systems which latter result in greater impact and wear of the wheels on the rail to the end that there is greater likelihood of breakage of the rail and injury to persons underneath. In one of its aspects, the invention may be regarded as an improvement on the rails forming the subject matter of the Bennington Patents Nos. 1,550,142 and 1,577,162 and the Wehr Patent No. 1,577,394.

The rails shown in these patents have proven quite satisfactory but they have the disadvantage that they are formed of high carbon steel which is not as ductile as structural or low carbon steel and does not give the desired assurance against breakage under the exacting conditions imposed by the demands of the users for increased load and speed of the carriers.

A more specific object is to provide a rail which is formed of low carbon steel or the like and which is provided on its lower flanges with wear and impact resisting treads formed of a different material and so fixed thereto as to give the rail long life.

The invention may be further briefly summarized as consisting in certain details of construction and combinations and arrangements of parts as well as steps of the method which will be described in the specification and set forth in the appended claims.

In the accompanying sheet of drawings,

Fig. 1 is a perspective view showing a portion of a rail embodying my invention; and

Fig. 2 is a perspective view on an enlarged scale of a portion of the rail illustrating how the tread is applied to the lower flange from fused metal or alloy deposited on the flange, and indicating the nature of the union which is obtained when the material forming the tread is applied by a welding operation.

Referring now to the drawing, 10 represents a monorail of an overhead monorail underslung carrier system the lower flanges of the rail being adapted to support the track wheels of the car-

riers in the well known manner. This rail is in this instance in the form of an I-beam, but whether it is in the form of an I-beam or a T-section (as when formed into a composite rail according to the teachings of the Wehr Patent No. 1,577,394), or in fact any other suitable section, is immaterial to the present invention. The rail here shown is provided with a web 11, upper flanges 12, and lower flanges 13 for the track wheels. The rail here shown is rolled in one piece with wide upper flanges to give lateral stiffness and greater resistance to bending under the weight of the carriers, the upper and lower flanges being tapered so that the section can be rolled on a regular beam mill.

Heretofore, to obtain a satisfactory wearing tread for the wheels, it has been customary to make the rails of fairly high carbon steel, as with the constructions disclosed in the Bennington and Wehr patents referred to above. However, high carbon steel has a tendency to break upon failure, caused by overload or the like, and since these systems are used largely in factories to handle material being fabricated, in all probability the carrier and load will fall upon workmen underneath. It is a feature of the present invention that the rail proper is made of low carbon steel or some similar ductile material which may bend but which will not break under overload, while the lower flanges of the rail are provided with hard, tough, flat wear-resisting treads for the wheels of the monorail carrier by progressively depositing along the top surfaces of the lower flanges suitable tread material in a fused state preferably from a weld wire and by a welding operation, (as by electric welding, wherein the wire is one of the electrodes) thus not only fusing the wire but also the adjacent portion of the flange so as to obtain an intimate and fused union between the deposited material and the steel flange of such a character that loosening of the tread in practice cannot occur.

In the drawing the treads provided on the lower flanges as just described are designated by the reference character 14, each tread being carried over the round corner of the flange and downwardly slightly so as to protect the edge of the flange from wear by the flanges of the wheels. After the tread is applied, it is ground so as to provide a flat top surface and a flat outer edge in line with the edge of the flange.

Depending upon the width of the tread, it may be applied and formed in one or more contiguous beads which, after the grinding operation, form in effect one continuous tread surface. Of

course, the thickness and width of the tread may be varied for rails of different sizes and in accordance with the operating conditions of the carrier system, such as the load transported by and the speed of operation of the carriers. As stated above, the tread is preferably formed and applied by an electric welder wherein the material forming the tread is the weld wire and constitutes one of the electrodes of the welding machine. When the tread is applied or formed in this manner, as will be seen by reference to Fig. 2, there is of course a molecular intermingling of the fused wire and the fused surface of the flange forming a union which cannot be loosened by use under any operating conditions. While, as stated above, the thickness and width of the tread may be varied as desired or as conditions require, I have obtained very good results by applying a tread having an average thickness of  $\frac{1}{16}$ " and a width of  $\frac{7}{16}$ " when applied to a 10" beam the base of which (measured across the lower flange) is  $3\frac{1}{4}$ ". These proportions of the tread and base of the beam are mentioned simply as one possibility and in no way in a limiting sense.

In forming the tread in the manner just stated, it is possible to obtain a tread having any desired strength, hardness, toughness, and ductility (a reasonable amount of the latter is desired). A Brinell hardness of from 300 to 500 is generally satisfactory. The above mentioned characteristics may be varied by the ingredients of the weld wire. Generally a mild steel wire is employed with a coating containing the elements desired to obtain an alloy which has the desired characteristics. I have obtained very good results using a structural steel rail having from .15% to .25% carbon content and depositing the tread on the lower flanges thereof in one or more beads with an electric welder employing a weld wire formed from mild steel with alloy ingredients in the coating of the wire containing small amounts of part or all of the following: carbon, manganese, silicon, chromium, nickel, boron. However, the particular alloy ingredients in the coating of the wire and the proportions thereof may be varied as found desirable. By the phrase "mild steel" as used throughout the appended claims, it is intended to cover low carbon steel, such as defined above or some similarly strong and ductile material.

Since the tread 14 is of less width than the flange to which it is secured and stands above the top surface of the adjoining portion of the flange, the present construction has all the advantages of the construction described and claimed in the Bennington Patent No. 1,550,142 as well as numerous advantages over the Bennington construction.

While I have shown the preferred construction and a method which operates satisfactorily, I do not desire to be confined to the same or to any particular proportions or ingredients so far as materials used in forming the tread are concerned but aim in my claims to cover all modifications which do not involve a departure from the spirit and the scope of my invention.

Having thus described my invention, I claim:

1. A rail for an overhead underslung carrier system comprising: an elongated body portion including flanges extending along the entire length of the lower part thereof, said body por-

tion having substantially the elongation characteristic of mild steel having approximately .15% to .25% carbon; and carrier wheel engaging tread portions on the upper surfaces of said flanges and extending the full length thereof, said tread portions being formed of hard wear resisting material having a Brinell hardness of approximately 300 to 500 deposited thereon in a fused state and welded or fused thereto.

10. 2. A rail for an overhead underslung carrier system comprising: an elongated body portion including flanges extending along the entire length of the lower part thereof, said body portion having substantially the elongation characteristics of mild steel having approximately .15% to .25% carbon; and carrier wheel engaging tread portions on the upper surfaces of said flanges and extending the full length thereof, said tread portions projecting downwardly over at least a

15. part of the free edges of said flanges and being formed of hard wear resisting material having a Brinell hardness of approximately 300 to 500 deposited thereon in a fused state and welded or fused thereto.

20. 3. A rail for an overhead underslung carrier system comprising: an elongated body portion including flanges extending along the entire length of the lower part thereof, said body portion having substantially the elongation characteristics of mild steel having approximately .15% to .25% carbon; and carrier wheel engaging tread portions on the upper surfaces of said flanges and extending the full length thereof, said flanges having rounded upper corners along the

25. free edges thereof and said tread portions extending downwardly over said rounded corners and being formed of hard wear resisting material having a Brinell hardness of approximately 300 to 500 deposited thereon in a fused state and welded or fused thereto.

30. 4. A rail for an overhead underslung carrier system comprising: an elongated body portion including flanges extending along the entire length of the lower part thereof; said body portion having substantially the elongation characteristics of mild steel having approximately .15% to .25% carbon; and carrier wheel engaging tread portions on the upper surfaces of said flanges and extending the full length thereof, the upper surfaces of said tread portions being raised above the upper surfaces of the flanges proper to form raised treads, and said tread portions being formed of hard wear resisting material having a Brinell hardness of approximately 300 to 500 deposited thereon in a fused state and welded or fused thereto.

35. 5. A rail for an overhead underslung carrier system comprising: a rolled elongated body portion I-beam in cross-section the upper flanges of which are wider than the lower flanges, said body portion having substantially the elongation characteristics of mild steel having approximately .15% to .25% carbon; and carrier wheel engaging tread portions on the upper surfaces of the lower flanges of said body portion and extending the full length thereof, said tread portions being formed of hard wear resisting material having a Brinell hardness of approximately 300 to 500 deposited thereon in a fused state and welded or fused thereto.

70. WILLIAM G. WEHR.